

3,676,139

### COLOR PHOTOGRAPHIC PRINTING PAPER

Hiroyuki Amano, Fumihiko Nishio, Nobuo Tsuji, and Kazuo Shirasu, Ashigara-Kamigun, Kanagawa, Japan, assignors to Fuji Shashin Film Kabushiki Kaisha (now Fuji Photo Film Co., Ltd.), Ashigara-Kamigun, Kanagawa, Japan

No Drawing. Filed Jan. 13, 1969, Ser. No. 790,846  
Claims priority, application Japan, Jan. 12, 1968,

43/1,669

The portion of the term of the patent subsequent to Oct. 26, 1988, has been disclaimed

Int. Cl. G03c 1/92, 1/84

U.S. Cl. 96—82

9 Claims

### ABSTRACT OF THE DISCLOSURE

A color photographic printing paper containing an ultraviolet absorber and a fluorescent brightening agent represented by the formulas



The present invention relates to a color photographic printing paper containing a fluorescent brightening agent and an ultraviolet absorber. More particularly, the invention relates to a color photographic printing paper having a photographic layer containing a water-soluble, fluorescent brightening agent having an anti-diffusion property to fluorescent-whitening and an ultraviolet absorber to prevent fading and stains caused by ultraviolet rays.

The whitening of photographic printing papers has previously been accomplished by a method comprising adding a fluorescent brightening agent to the baryta layer of a baryta paper. However, even if a baryta-coated paper is whitened by the aforesaid conventional method, the whitening effect is lost in color photographic printing paper, since such papers must also contain a compound capable of absorbing ultraviolet rays, such as, ultraviolet absorber and a coupler.

Therefore, various suggestions have been made to supplement the whitening effect thus lost. For example, there has been proposed a method in which a water-soluble fluorescent brightening agent is incorporated in a processing solution and a gelatin-containing layer is processed by

the solution to dye the gelatin with the fluorescent brightening agent. However, this method has the disadvantage that it is difficult to dye selectively a necessary layer with a fluorescent brightening agent. In addition, an additional processing bath containing the fluorescent brightening agent is required.

There has also been proposed a direct-addition method, in which a fluorescent brightening agent is added directly as an aqueous solution or an organic solvent solution

10 thereof to an emulsion or a dispersion for a photographic silver halide emulsion layer or to a supplemental layer. An indirect method has been proposed, in which a fluorescent brightening agent is dissolved in a solvent having a high boiling point (or a mixture of a high boiling solvent and 15 an auxiliary solvent), the solution dispersed in an aqueous gelatin solution, and this dispersion added to a photographic light-sensitive emulsion.

However, since the known fluorescent brightening agents are usually low molecular weight compounds, when they 20 are incorporated in photographic emulsion layers or sup-

plemental layers, the greater part of the fluorescent brightening agents is diffused out during processing and washing, whereby the whitening effect thereof is weakened.

Various proposals have been made to avoid the above 40 disadvantages of the prior art processes. For instance, there has been proposed a method in which a substituent capable of improving dyability is introduced into gelatin. For example, polyvinyl pyrrolidone (Japanese Pat. No. 7127(1959)) and poly-N-vinyl-5-methyl-3-oxazolidinone (Japanese Pat. No. 22,065(1964)), each being capable of 45 being readily dyed by a fluorescent brightening agent, have been dispersed in an aqueous gelatin solution and then dyed by a fluorescent brightening agent. However, even by employing such methods, the diffusion of the fluorescent brightening agent employed has yet to be sufficiently prevented and the whitening effect of the agent is 50 still considerably degraded during photographic processing and washing.

The inventors have previously found that as disclosed in their U.S. application Ser. No. 720,344, filed Apr. 10, 1968 now Pat. No. 3,556,081, the aforesaid disadvantages are overcome to the same extent by using, as the fluorescent brightening agent a compound having a repeating unit represented by one of the following general formulas:



wherein  $R_0$  and  $R_2$  each represents a hydrogen atom, an alkyl group having 1-8 carbon atoms, an aryl group having 6-12 carbon atoms, a hydroxylalkyl group having 2-4 carbon atoms, or a substituted derivative thereof, a sulfoalkyl group having 1-4 carbon atoms, or an alkali metal salt or ammonium salt thereof;  $R_1$  represents a halogen atom,  $—OR$ ,  $—SR$ ,



or



wherein R and R' each represents a hydrogen atom, an alkyl group having 1-12 carbon atoms, a hydroxylalkyl group having 1-12 carbon atoms, a sulfoalkyl group (or an alkali metal salt or an ammonium salt thereof) a carboxylalkyl group (or an alkali metal salt or an ammonium salt thereof), or an alkyl group, an aryl group having 6-18 carbon atoms, a hydroxy-, carboxy- or sulfonic acid-derivative thereof, or an alkali metal salt or an ammonium salt thereof, a cycloalkyl group having 2-10 carbon atoms, or a substituted cycloalkyl group; and wherein A represents an alkylene group having 4-5 carbon atoms or an alkylene group containing a heterocyclic atom or a heterocyclic atomic group; Y represents an alkylene group having 2-10 carbon atoms, a substituted alkylene group having 2-10 carbon atoms, an allylene group having 6-18 carbon atoms or a substituted allylene group having 6-18 carbon atoms; Z represents a divalent heterocyclic atom or atomic group; M represents an alkali metal atom or  $NH_4$ ; X represents OH, Cl or  $NH_2$ , m is 0 or 1 and n is 5 to 120. That is, the fluorescent brightening agent is less diffused out during photographic processing or washing when incorporated in a photographic emulsion layer or a supplemental layer. Further, it has been found that this is resistant to staining when exposed to ultraviolet rays. Furthermore, these fluorescent brightening agents have been found to be excellent in fluorescent intensity and wave length.

It is also known to incorporate an ultraviolet absorbent in the photographic emulsion layer or an upper layer applied on that photographic emulsion layer for improving the fade-resistance of color images. The known ultraviolet absorbents are those absorbing ultraviolet rays having wave lengths of 300-400  $m\mu$ . It is also known that a ultraviolet absorbent capable of absorbing ultraviolet rays having wave lengths as long as possible is more effectively employed.

However, when the absorption edge of known ultraviolet absorbents extends across 400  $m\mu$ , the ultraviolet absorbent becomes yellow in color, and thus influences adversely the whiteness of the printing paper.

It is therefore, an object of this invention to provide a color photographic printing paper wherein the above coloration, resulting from the use of an ultraviolet absorbent, is substantially avoided.

It is a further object of this invention to provide a color photographic printing paper which has been whitened by a fluorescent brightening agent, wherein fading of the color upon exposure to light is reduced by the addition of an ultraviolet absorbent, without adversely affecting the whiteness thereof.

A further object of this invention is the provision of a color photographic printing paper containing an ultraviolet absorbent and a fluorescent whitening agent which is not subject to the aforesaid disadvantages.

The aforesaid objects of the present invention can be achieved by incorporating a fluorescent brightening agent having at least one repeating unit represented by the general Formula I or II in at least one photographic layer of a color photographic printing paper, said layer containing an ultraviolet absorbent, and photographic layers

present at the side of said photographic layer containing the ultraviolet absorbent and opposite to the support side of the paper.

For example, in one embodiment of a color photographic printing paper, there are provided on a support, a baryta layer, a blue-sensitive emulsion layer containing a yellow coupler, an intermediate layer, a green-sensitive emulsion layer containing a magenta coupler, an intermediate layer, a red-sensitive emulsion layer containing a cyan coupler, and a protective layer in that order. The ultraviolet absorbent is incorporated in the intermediate layer between the cyan coupler-containing emulsion layer and the magenta coupler-containing emulsion layer and the fluorescent brightening agent is incorporated in the protective layer.

The fluorescent brightening agent used in the present invention is a high molecular weight compound having the repeating unit of the general Formula I or II as mentioned above. The ultraviolet absorbent used in this invention may be, for instance,

(1) A benzotriazole derivative represented by the following general formula:



wherein  $R_1'$ ,  $R_2'$ , and  $R_3'$  each represents a hydrogen atom, a halogen atom, a nitro group, an alkyl group, an aromatic group, or a heterocyclic ring;

(2) A benzophenone derivative represented by general Formula IV



wherein  $R_1''$  and  $R_2''$  represent an alkyl group and  $R_3''$  and  $R_4''$  represent a hydrogen atom or an alkoxy group; or

(3) A thiazolidone derivative, represented by general Formula V



wherein  $R'''$  represents a hydrogen atom, an alkyl group, a cycloalkyl group, an aralkyl group, or an aryl group;  $R_1'''$  represents an aryl group or a pyridyl group; and Q represents an imino group, a thiazole derivative, a cinnamic acid ester derivative, an oxazole derivative, an imidazole derivative, an oxadiazole derivative, thiadiazole derivative, a thiophene, benzalazine derivative, or a bis-hydroxyarylamide compound.

The ultraviolet absorbent may be incorporated in the coating composition for photographic layer as (1) an emulsified dispersion in an aqueous gelatin solution, (2) a solution thereof in a high boiling solvent or a mixed solvent containing a high boiling solvent and a low boiling solvent or (3) an aqueous alkaline solution thereof.

The high molecular weight fluorescent brightening agents employed in the present invention and methods of preparing them are described completely in copending U.S. application Ser. No. 720,344, filed Apr. 10, 1968.

As set forth therein, the high molecular weight compounds having the repeating unit represented by aforesaid general Formula I or II are generally prepared by dissolving or dispersing in a solvent, such as water or

dimethylformamide, one mol of an S-triazine-stilbene derivative having the general formula



wherein X represents a halogen atom or an alkoxy group having 1-4 carbon atoms and R<sub>0</sub>, R<sub>1</sub> and M are as indicated above, and about one mol of a diamino compound represented by general Formula IV or V as follows:



or



wherein R<sub>2</sub>, Y, Z, and m are as indicated above, reacting this mixture at a temperature of from about 50 to 150° C. with the addition of 2-2.4 mols of an aqueous sodium hydroxide solution. In addition high molecular weight compounds of this invention may be prepared by other methods and may be employed in this invention.

The bis-S-triazine-stilbene derivative described by general Formula III may be prepared by conventional methods, as shown in "The Journal of the Society of Organic Chemistry, Japan," vol. 20, 64 (1962).

For example, the derivative may be prepared by reacting 2 mols of cyanuric chloride with one mole of a derivative of 4,4'-diaminostilbene-2,2'-disulfonate represented by the general formula



wherein R<sub>0</sub> and M are as set forth above, at a temperature of about -5° C. to 10° C. The compound thus obtained is reacted with 2 mols of a nucleophilic agent illustrated by the formula HR<sub>1</sub>, wherein R<sub>1</sub> is as set forth above, at a temperature of from about 0 to 20° C.

Some examples of R<sub>0</sub>, R, Y, and Z in the repeating unit (I) or (II) of the high molecular weight compounds of this invention are as follows:

R<sub>0</sub> and R<sub>2</sub> may be, for example: -H, -CH<sub>3</sub>, -C<sub>2</sub>H<sub>5</sub>, -C<sub>3</sub>H<sub>7</sub>, -CH<sub>2</sub>CH(CH<sub>3</sub>)<sub>2</sub>,



-CH<sub>2</sub>CH<sub>2</sub>OH, -CH<sub>2</sub>CH<sub>2</sub>CH<sub>2</sub>OH, -CH<sub>2</sub>CH<sub>2</sub>OCH<sub>3</sub>, -CH<sub>2</sub>CH<sub>2</sub>OCH<sub>5</sub>, -CH<sub>2</sub>-SO<sub>3</sub>M' (where M' represents H, Na, K or NH<sub>4</sub>), -(CH<sub>2</sub>)<sub>3</sub>-SO<sub>3</sub>M', -(CH<sub>2</sub>)<sub>4</sub>SO<sub>3</sub>M', and the like.

R<sub>1</sub> may be for example:



-N(CH<sub>3</sub>)<sub>2</sub>, -N(C<sub>2</sub>H<sub>5</sub>)<sub>2</sub>, -N(C<sub>4</sub>H<sub>9</sub>)<sub>2</sub>  
-NHCH<sub>2</sub>CH<sub>2</sub>OH, -N(CH<sub>2</sub>CH<sub>2</sub>OH)<sub>2</sub>-NH(CH<sub>2</sub>)<sub>p</sub>SO<sub>3</sub>M'

(where M'=H, Na, K or NH<sub>4</sub> and P=1, 2, 3, 4)

5 -NH(CH<sub>2</sub>)<sub>p</sub>COOM', -N

H

, -N

H

, -N

H

O

10 -N

H

S

, -NH-

, -NH-

CH<sub>3</sub>

-NH-

, -NH-

COOM'

-NH-

SO<sub>3</sub>M'

, -NH-

OH

-NH-

Cl

, -

SO<sub>3</sub>M'

, -

COOM'

25 -N

, -NH-

, -NH-

S

N

(where M'=H, Na, K or NH<sub>4</sub> and P=1, 2, 3 or 4)

As examples of Y may be mentioned:

30 -CH<sub>2</sub>-CH<sub>2</sub>-(q=2-10), -CH<sub>2</sub>-CH-

CH<sub>3</sub>

, -CH<sub>2</sub>-C-

CH<sub>3</sub>

-CH<sub>2</sub>CH<sub>2</sub>OCH<sub>2</sub>CH<sub>2</sub>-, -CH<sub>2</sub>CH-

CH<sub>3</sub>

-CH<sub>2</sub>CH-

OH

, -CH<sub>2</sub>CH-

COOH

-CH<sub>2</sub>-

, -CH<sub>2</sub>-

, -CH<sub>2</sub>-

CH<sub>2</sub>-

-CH<sub>2</sub>-

, -CH<sub>2</sub>-

, -CH<sub>2</sub>-

COOM'

45 -CH<sub>2</sub>-

COOM'

, -CH<sub>2</sub>-

COOH<sub>3</sub>

CH<sub>3</sub>

50 -CH<sub>2</sub>-

, -CH<sub>2</sub>-

-CH<sub>2</sub>-

COOM'

SO<sub>3</sub>M'

55 -CH<sub>2</sub>-

-CH<sub>2</sub>-

-

60 -CH<sub>2</sub>-

-CH<sub>2</sub>-

O-

65 -CH<sub>2</sub>-

SO<sub>3</sub>M'

-CH<sub>2</sub>-

C

CH<sub>3</sub>

70 -CH<sub>2</sub>-

-CH<sub>2</sub>-

-

75 -CH<sub>2</sub>-

-CH=CH-



(where  $M' = H, Na, K$  or  $NH_4$ ),  $Z$  may be exemplified by  $O, S$ , and  $SO_2$ .

Typical examples of compounds included in general Formulas I or II which may be used in this invention are as follows:

(1)



(2)



(3)



(4)



(5)



(6)



(7)





(14)



It will, of course, be understood, that the number of repeating units (represented by  $n$ ) set forth in the foregoing examples may vary to some extent, the narration in some instances being up to about  $\pm 20$  repeating units.

These compounds may generally be prepared by the methods described above, but an example will be given in detail for Compound 1.

A solution of 14.7 parts by weight of cyanuric chloride in 80 parts of acetone is dispersed in a slurry of 240 parts by weight of ice water, and the dispersion is maintained at about 0-3° C. To the dispersion there is added dropwise 16.5 parts of sodium 4,4'-diaminostilbene-2,2'-disulfonate as a 10% aqueous solution. During the addition, hydrochloric acid is formed in the system, and an aqueous solution of sodium carbonate is added dropwise (4.2 parts by weight sodium carbonate and 50 parts by weight water) so that the pH of the system is in the range of 4-5. The system is, thereafter, stirred for about 30 minutes at about 0-5° C., and 7.5 parts of aniline is further added to the reaction mixture. Thereafter, the temperature of the system is increased to 20° C. and an aqueous solution of sodium carbonate (4.2 parts by weight sodium carbonate and 60 parts by weight water) is added gradually to the system.

After conducting the reaction for about 3 hours at the same temperature, 2.4 parts by weight of ethylenediamine is added to the reaction mixture, and the reaction temperature is increased to 100° C. The reaction mixture is stirred for 2 hours at 100° C. Upon filtering the reaction mixture after cooling, Compound 1 is obtained.

The compound thus obtained is soluble in a dimethylformamide-water 1:1 solvent, and the intrinsic viscosity of the compound in the same solvent is 0.32 at 30.0° C.

Likewise, typical examples of ultraviolet absorbents which may be used in the present invention are as follows:

(15)



(16)



(17)



(18)



(19)



(20)

15

20

25

30

35

40

45

50

60

65

70

75

 $(n \geq 5)$ 

Proportions of high molecular weight fluorescent brightening agent which may be employed in the printing papers brightening agent of this invention range from 0.5-10 mg./100 cm.<sup>2</sup> and those of the ultraviolet absorbent range from 2-20 mg./100 cm.<sup>2</sup>

Almost all conventionally known fluorescent brightening agents are simultaneously ultraviolet absorbents. The fluorescent brightening agent may be added to the system by either the direct or the indirect method as set forth above.

When known fluorescent brightening agents are added to an uppermost layer of a photographic light sensitive color printing paper by the indirect method, that layer frequently becomes subject to damage by external impact or friction. Further, the layer may become sticky, particularly when mounted in an album as a result of solvent action. Therefore, when such conventional fluorescent brightening agents are employed, they must be incorporated in a photographic layer other than the uppermost layer.

However, when the fluorescent brightening agents of this invention are employed, it is possible to incorporate them in the uppermost layer without incurring such disadvantages. Hence the fluorescent brightening agents of this invention may be incorporated in the uppermost layer to be effectively utilized as an ultraviolet absorbent.

Of course, it will be understood that the high molecular weight compound of this invention may be incorporated in any layer to effect ultraviolet preventing and fluorescent brightening action.

The term "photographic emulsion" in this application is defined to mean the usual gelatino silver halide light-sensitive emulsions, but synthetic resins such as polyvinyl alcohol and polyvinyl acetate may be effectively employed as protective colloids for the photographic emulsion, in addition to gelatin, in this invention.

In the present invention, the order of the photographic layers, as well as the number of the layers, may be varied as is well known in the art. Moreover, the ultraviolet absorbent of this invention may be incorporated in any layer except the protective, or uppermost layer. Further,

## 13

the fluorescent brightening agents of this invention may be incorporated either in the layer containing the ultraviolet absorbent or in a layer positioned at the side of the ultraviolet absorbent-containing layer opposite to the side of support.

The invention may be illustrated by the following typical examples which exemplify various combinations of the water-soluble high molecular weight fluorescent brightening agent and the ultraviolet absorbent, although it will be understood that the invention shall not be limited thereby.

## EXAMPLE 1

Compound 1, supra, was employed as the high molecular weight fluorescent brightening agent, and the effect thereof was measured. A color photographic printing paper consisting of a support, a baryta paper, a blue-sensitive emulsion layer containing 3,5-dicarboxy- $\alpha$ -(4-stearoylamido-benzoyl)acetanilide as the yellow coupler, an intermediate layer, a green-sensitive emulsion layer containing 1,3-sulfo-4-phenoxyphenyl)-3-stearoyl-5-pyrazolone as the magenta coupler, an ultraviolet absorption layer containing Compound 17, supra, as the ultraviolet absorbent, a red-sensitive emulsion layer containing N-n-octadecyl-1-hydroxy-4-sulfo-2-naphthamide as the cyan coupler, and a protective layer, in this order, was prepared and designated "color photographic printing paper A." In addition, a photographic color printing paper having the same photographic layers as above in the same order, but containing no ultraviolet absorbent in the intermediate layer between the green-sensitive emulsion layer and the red-sensitive emulsion layer was prepared, and is designated "color photographic printing paper B." Compound 1 was incorporated in each layer of the photographic color printing paper A

## 14

agent of this invention was incorporated in the uppermost layer, the use of a whitening procedure for the baryta layer was unnecessary.

## EXAMPLE 2

To a baryta-coated paper was applied a blue-sensitive silver iodobromide emulsion containing 3,5-dicarboxy- $\alpha$ -(4-stearoylamido-benzoyl)acetanilide as a yellow coupler. The coupler was added as an aqueous alkaline solution thereof. Thereafter, a green-sensitive silver chlorobromide emulsion containing 1 - (3-sulfo-4-phenoxy)-3-stearoyl-5-pyrazolone as a magenta coupler was applied to the blue-sensitive layer. An ultraviolet absorbent, one of the Compounds 15-23, supra, was dispersed by emulsification in dibutyl phthalate and the dispersion was added to a red-sensitive silver chlorobromide emulsion together with N-n-octadecyl-1-hydroxy-4-sulfo-2-1-naphthamide as a cyan coupler, and the resulting emulsion was applied to the green-sensitive emulsion layer. Over this layer, there was further formed a protective layer in a thickness of 2.0 microns. This protective layer was formed by adding slowly a 4% dimethyl formamide-water solution of one of the Compounds 1-14, supra, as a high molecular weight fluorescent brightening agent or Compound 24 or 25 having the structural formulas as shown below, well-known fluorescent brightening agent, to an aqueous gelatin solution and applying the resulting mixture in a thickness of 5 mg./100 cm.<sup>2</sup> followed by drying.

The color photographic printing paper thus prepared was developed in a developer containing N-ethyl-N- $\beta$ -hydroxyethyl-p-phenylenediamine and thereafter subjected to stop fixing, washing, bleach fixing, washing, hardening, washing, and drying. The whiteness of the printing paper thus processed is shown in the following table.

(24)



(25)



and photographic color printing paper B at a level of 5 mg./100 cm.<sup>2</sup>, and the thus prepared color photographic processing. The whiteness of the color photographic printing papers thus processed is shown in the following table, in which the whiteness is shown by photographic density of the yellow component in the unexposed portions of the processed printing papers.

## DENSITY OF YELLOW COMPONENT IN UNEXPOSED PORTION

| Layer to which compound is added                    | Printing paper |      | Compound |
|-----------------------------------------------------|----------------|------|----------|
|                                                     | A              | B    |          |
| Protective layer                                    | 0.06           | 0.05 | 15       |
| Cyan layer                                          | 0.09           | 0.08 | 16       |
| Ultraviolet absorbing layer (or intermediate layer) | 0.10           | 0.08 | 17       |
| Magenta layer                                       | 0.11           | 0.09 | 18       |
| Intermediate layer                                  | 0.11           | 0.09 | 19       |
| Yellow layer                                        | 0.11           | 0.09 | 20       |
| Baryta layer                                        | 0.12           | 0.09 | 21       |
| No additive                                         | 0.12           | 0.10 | 22       |
|                                                     |                |      | 23       |

From the above results, it can be seen that the effect of the fluorescent brightening agent was most remarkable when it was incorporated in the uppermost layer, and that the effect became less as it was incorporated in those layers nearer the support. Also, it should be noted that, when the high-molecular weight fluorescent brightening

## DENSITY OF YELLOW COMPONENT OF UNEXPOSED PORTION

| Ultraviolet<br>absorbent<br>brightening<br>agent | Compound |      |      |      |      |      |      |      |      |
|--------------------------------------------------|----------|------|------|------|------|------|------|------|------|
|                                                  | 15       | 16   | 17   | 18   | 19   | 20   | 21   | 22   | 23   |
| Compound:                                        |          |      |      |      |      |      |      |      |      |
| 1                                                | 0.06     | 0.06 | 0.06 | 0.07 | 0.06 | 0.07 | 0.07 | 0.07 | 0.07 |
| 2                                                | 0.06     | 0.06 | 0.06 | 0.07 | 0.06 | 0.07 | 0.07 | 0.07 | 0.07 |
| 3                                                | 0.06     | 0.06 | 0.06 | 0.07 | 0.06 | 0.07 | 0.07 | 0.07 | 0.07 |
| 4                                                | 0.06     | 0.06 | 0.06 | 0.07 | 0.06 | 0.07 | 0.07 | 0.07 | 0.07 |
| 5                                                | 0.06     | 0.06 | 0.06 | 0.07 | 0.06 | 0.07 | 0.07 | 0.07 | 0.07 |
| 6                                                | 0.06     | 0.06 | 0.06 | 0.07 | 0.06 | 0.07 | 0.07 | 0.07 | 0.07 |
| 7                                                | 0.06     | 0.06 | 0.06 | 0.07 | 0.06 | 0.07 | 0.07 | 0.07 | 0.07 |
| 8                                                | 0.06     | 0.06 | 0.06 | 0.07 | 0.06 | 0.07 | 0.07 | 0.07 | 0.07 |
| 9                                                | 0.06     | 0.06 | 0.06 | 0.07 | 0.06 | 0.07 | 0.07 | 0.07 | 0.07 |
| 10                                               | 0.06     | 0.06 | 0.06 | 0.07 | 0.06 | 0.07 | 0.07 | 0.07 | 0.07 |
| 11                                               | 0.06     | 0.06 | 0.06 | 0.07 | 0.06 | 0.07 | 0.07 | 0.07 | 0.07 |
| 12                                               | 0.06     | 0.06 | 0.06 | 0.07 | 0.06 | 0.07 | 0.07 | 0.07 | 0.07 |
| 13                                               | 0.06     | 0.06 | 0.06 | 0.07 | 0.06 | 0.07 | 0.07 | 0.07 | 0.07 |
| 14                                               | 0.06     | 0.06 | 0.06 | 0.07 | 0.06 | 0.07 | 0.07 | 0.07 | 0.07 |
| 24                                               | 0.11     | 0.11 | 0.11 | 0.12 | 0.11 | 0.12 | 0.12 | 0.12 | 0.12 |
| 25                                               | 0.11     | 0.11 | 0.11 | 0.12 | 0.11 | 0.12 | 0.12 | 0.12 | 0.12 |
| No compound                                      | 0.12     | 0.12 | 0.12 | 0.13 | 0.12 | 0.13 | 0.13 | 0.13 | 0.13 |

As can be clearly seen from the above results, when a high molecular fluorescent brightening agent of this invention was incorporated in the uppermost layer of the color photographic printing paper, a very remarkable

whitening effect was obtained. On the other hand, when the conventional fluorescent brightening agent, Compound 24 or 25 was employed, the fluorescent brightening agent was diffused out during photographic processing to reduce the whitening effect. Further, due to the fact that the color photographic printing papers of this invention have an ultraviolet absorbent-containing layer, their light fastness quality is also excellent.

What is claimed is:

1. A color photographic printing paper comprising a 10 support paper containing an ultraviolet absorbent and a compound selected from the group consisting of compounds having the formulas



wherein  $R_0$  and  $R_2$  are each a member selected from the group consisting of a hydrogen atom, an alkyl group having 1-8 carbon atoms, an aryl group having 6-12 carbon atoms, a hydroxyalkyl group having 2-4 carbon atoms, a substituted hydroxy alkyl group having 2-4 carbon atoms, a sulfoalkyl group having 1-4 carbon atoms, and alkali metal salts and ammonium salts thereof;  $R_1$  is a member selected from the group consisting of a halogen atom,  $-OR$ ,  $-SR$ ,



and



wherein R and R' are each a member selected from the group consisting of a hydrogen atom, an alkyl group having 1-12 carbon atoms, a hydroxyalkyl group having 1-12 carbon atoms, a sulfoalkyl group, an alkali metal salt of said sulfoalkyl group, an ammonium salt of said sulfoalkyl group, a carboxyalkyl group, an alkali metal salt of said carboxyalkyl group, an ammonium salt of said carboxyalkyl group, an alkyl group, an aryl group having 6-18 carbon atoms, a hydroxyl derivative of said aryl group, a carboxyl derivative of said aryl group, a sulfonic acid derivative of said aryl group, an alkali metal salt of each said derivative, an ammonium salt of such said derivative, a cycloalkyl group having 2-10 carbon

atoms, and a substituted cycloalkyl group; A is a member selected from the group consisting of an alkylene group having 4-5 carbon atoms, an alkylene group containing a heterocyclic atom, and an alkylene group containing a heterocyclic atomic group; Y is a member selected from the group consisting of an alkylene group having 2-10 carbon atoms, a substituted alkylene group having 2-10 carbon atoms, an allylene group having 6-18 carbon atoms and a substituted allylene group having 6-18 carbon atoms, Z is a member selected from the group consisting of a divalent heterocyclic atom and a divalent heterocyclic atomic group; M is a member selected from the group consisting of an alkali metal atom and  $\text{NH}_4$ ; X is

a member selected from the group consisting of hydroxyl, chloro and amino;  $m$  is 0 or 1, and  $n$  is 5 to 120.

2. The color photographic printing paper as claimed in claim 1 wherein said ultraviolet absorbent is a member selected from the group consisting of a benzotriazole, a benzophenone and a thiazolidone.

3. The color photographic printing paper as recited in claim 2 wherein the amount of said compound is 0.5-10 mg./100 cm.<sup>2</sup> and the amount of said ultraviolet absorbent is 2-20 mg./100 cm.<sup>2</sup>.

4. The color photographic printing paper as recited in claim 1 wherein said printing paper comprises a layer containing said ultraviolet absorbent and a layer containing said compound, the layer containing said ultraviolet absorbent being positioned between said compound-containing layer and said support paper.

5. The color photographic printing paper as recited in claim 4, wherein said compound is incorporated in the uppermost protective layer of the printing paper.

6. The color photographic printing paper as recited in claim 1 wherein said ultraviolet absorbent and said compound are both present in a single layer.

7. The color photographic printing paper as recited in claim 1 wherein said ultraviolet absorbent is incorporated in a layer below the uppermost layer.

8. The color photographic paper as recited in claim 6 wherein said ultraviolet absorbent and said compound are present in a layer beneath the uppermost layer.

9. The color photographic printing paper as claimed in claim 1 wherein said compound is selected from the group consisting of







## References Cited

## UNITED STATES PATENTS

2,933,390 4/1960 McFall et al. ----- 96—84

NORMAN G. TORCHIN, Primary Examiner

E. C. KIMLIN, Assistant Examiner

U.S. Cl. X.R.

96—48